

A. C. McCLOSKEY.  
PHOTOGRAPHIC PAPER.  
APPLICATION FILED MAR. 12, 1915.

1,213,925.

Patented Jan. 30, 1917.

FIG. 1.



FIG. 2.



FIG. 3.

WITNESS:

Bob Kitchel.

INVENTOR

Alfred C. McCloskey  
BY

Augustus B. Stoughton  
ATTORNEY

# UNITED STATES PATENT OFFICE.

ALFRED C. McCLOSKEY, OF PHILADELPHIA, PENNSYLVANIA, ASSIGNOR TO PROCESS  
PAPER MANUFACTURING COMPANY, A CORPORATION OF DELAWARE.

## PHOTOGRAPHIC PAPER.

1,213,925.

Specification of Letters Patent. Patented Jan. 30, 1917.

Application filed August 12, 1915. Serial No. 45,226.

*To all whom it may concern:*

Be it known that I, ALFRED C. McCLOSKEY, a citizen of the United States, residing at the city of Philadelphia, in the county of 5 Philadelphia and State of Pennsylvania, have invented a certain new and useful Photographic Paper, of which the following is a specification.

There are photographic papers on the 10 market and finishing processes in use by which prints in appropriately colored lines on a white or substantially white background can be produced from tracings or the like by exposure either to the sun's rays 15 or to artificial light. The prints, like the tracings, have dark images on white or substantially white grounds and no negative is used. Such processes are characterized by the use of a light sensitive coating containing, 20 perhaps, among other things an organic substance as gum, and ferric salt or salts which upon exposure to light are converted to the ferrous state or condition, and that potassium ferrocyanid is used as a developer, the 25 use of staining solutions being optional, and that sulfuric acid is the clearing solution. In reference to such papers it has been said that they are provided with such sensitized coatings as are normally insoluble in the 30 clearing solutions, but are rendered soluble by exposure, but whether this be absolutely accurate or not is perhaps not material since the above description sufficiently identifies the class of photographic papers upon which 35 the present invention is an improvement. However, in the finishing process or operation, such known paper must be wet only on the front or face, otherwise the back of the paper will be stained or discolored by the 40 solutions used or by impurities therein, and these stains and discolorations are not only unsightly in themselves but also frequently show through from the front.

It is the principal object of the present 45 invention to provide improved photographic paper of the general kind referred to and which can be immersed in or wet upon both sides with finishing solutions without danger of discoloration or stains on the back, where- 50 by the process of finishing the prints is facilitated and the production of prints with clean backs is insured.

Inasmuch as my invention is an improve-

ment in an existing art, I believe that it can be best explained by describing it in connection with a known process and means. For this purpose and not as a limitation or restriction of the application or use of the invention, I will refer to "Pellet" paper and to the "Pellet" process in the following description: "Pellet" paper is coated on one face with a coating containing gum arabic, tartaric acid and ferric chlorid. The developer may be potassium ferrocyanid and the clearing solution may be sulfuric acid. 65 Staining solutions may, of course, be employed when it is desired to produce, for example, black instead of blue lines on a white ground from a tracing or the like in which the lines are black and the ground is 70 white.

In Pizzighelli's modification of the "Pellet" process the coating that is applied to one side of the paper contains gum arabic, ammonium ferric citrate, and ferric chlorid. 75 The finishing solutions are the same.

My photographic paper differs from and is an improvement upon "Pellet's" or like or equivalent paper in that, while its face is generally or substantially the same as 80 those known papers, its back is provided with a coating soluble in or rendered removable by the clearing solution, and inert in or impermeable to or not permanently affected by not only the developing solution 85 but also the staining and fixing solutions where the two latter are employed for producing black or dark instead of blue or like lines. Photographic paper of my invention is, as heretofore, provided upon the face 90 with a ferric light sensitive coating, but it is additionally provided upon the back with a coating soluble in or removable by the clearing solution, whereby the paper, after printing, can be immersed in all the solutions used, and will present, when finished, 95 a clean back free from discolorations or stains.

In the accompanying drawings which are diagrammatic representations, Figure 1 is a 100 front view. Fig. 2, is a transverse sectional view of paper embodying features of the invention, and Fig. 3, is a sectional view, embodying a modification.

In the drawings 2, is a light sensitive coating containing, among other things, ferric

salts and this coating may be substantially the coating of the type above described as Pellet's and Pizzighelli's. The coating 1<sup>a</sup> is characterized as being ferrous and it may be 5 produced by making it originally the same as the coating 2, that is, ferric, and exposing it to light to reduce it to the ferrous state. The coating 1<sup>a</sup> is substantially the same as the coating 1, that is ferrous, and it may be 10 made by incorporating initially ferrous salts into it instead of ferric salts, as is done by Pellet and Pizzighelli. After the face of this paper has been exposed to light under a tracing, or the like, it is developed with 15 potassium ferrocyanid, stained or not as may be required with appropriate staining solutions that are well known and cleared with a sulfuric acid solution. Of course in the process the print is washed as usual 20 with water. The finished print will have a white back, a white ground and an image in dark lines.

One way of making paper embodying features of my invention is to provide both 25 sides of the paper with a ferric light sensitive coating and to primarily expose one side to convert the ferric coating to a ferrous non-light sensitive coating, thus producing the back. After such paper is printed upon 30 the ferric light sensitized side or face, the part of the coating on the face which has been exposed is therefore ferrous and the same as the coating on the back. In consequence the coating on the back and the 35 part of the coating on the face which has been exposed will respond and behave alike in the finishing solutions—potassium ferrocyanid, the developer, sulfuric acid the clearing solution, and staining solutions if 40 employed—so that the paper can be immersed therein or wet therewith without danger of staining or discoloring the back, because any stains or discolorations produced on the back by reason of the character 45 of the solutions used or of impurities therein are removed by the action of the clearing solution.

Another way of making photographic paper embodying features of the invention is 50 to provide the back of the paper with a coating initially ferrous and removable by or soluble in the clearing solution. This coating is not light sensitive and is not primarily exposed, but performs the function of preventing stains and discolorations on the back 55 because it protects the same and is only removed by the clearing solution.

The word paper is used herein in its ordinary sense and so as to include linen, 60 tracing-cloth, or any equivalent material, and the word tracings includes plates, films, transparencies and the like.

From the foregoing description it is obvious that changes may be made in details 65 by substituting equivalents in the applica-

tion of the invention to different known papers and printing processes, so that the invention is not limited in those respects nor otherwise than as the claims may require.

What I claim is:

1. Photographic paper for producing prints having dark images on light grounds from tracings and the like, provided upon the face with a light sensitive coating containing ferric salts and provided upon the 70 back with a coating containing ferrous salts and removable by the clearing solution, whereby the paper after printing can be immersed in or wet on both sides with the appropriate solutions tending to stain it and 75 will, when finished, present a clean back free from discolorations or stains.

2. Photographic paper for producing prints having dark images on light grounds from tracings and the like, provided upon 85 each face with a coating of which the coating on the face contains ferric salts and of which the coating on the back has been primarily exposed to reduce ferric salts to ferrous salts, whereby the coating on the 90 back comes off in the clearing solution to provide a clean stainless back.

3. Photographic paper for producing prints from tracings and the like provided on its back with a coating which does not 95 produce images and which is removable by the clearing solution, substantially as described.

4. Photographic paper for producing prints having dark images on light grounds 100 from tracings and the like, provided upon one face with a light sensitive coating and upon the other face with a non-printing protective coating having the same behavior in respect to the finishing solutions as have the 105 portions of the light sensitive coating after they have been exposed in printing, substantially as described.

5. Photographic paper having on the back thereof a non-printing coating impermeable to stains from the finishing solutions and removable by the clearing solution. 110

6. A photographic paper having on the face a sensitizing coating adapted to be 115 finished by solutions which produce stains, and having on the back a protective coating entirely removable by the clearing solution.

7. Photographic paper for producing light ground dark line prints directly from 120 tracings and having on the face a sensitizing coating and requiring protection for the back, and having on the back a non-developing protective coating of substantially the same characteristics as are imparted to the 125 face coat by light exposure and entirely removable by the clearing solution, substantially as described.

8. Photographic paper for producing from tracings and the like prints having 130

dark lines or marks where the tracing has dark lines or marks and having a light ground where the tracing has a light ground and adapted after immersion in the finishing solutions to present on the back a paper surface free from stains and images.

9. A photographic paper covered on the

back with a non-developing coating the same as that part of the coating on the face which after printing is inert in the developing 10 solutions and removable by the clearing solution.

ALFRED C. McCLOSKEY.